

## UNITED STATES PATENT OFFICE

JAMES F. WALSH, OF EAST ORANGE, AND THOMAS E. ALCORN, OF MAPLEWOOD, NEW JERSEY, ASSIGNEES TO CELLULOID CORPORATION, A CORPORATION OF NEW JERSEY

## PLASTIC FILM OR SHEET CONTAINING CELLULOSE NITRATE

No Drawing.

Application filed November 24, 1928. Serial No. 321,759.

This invention relates to the preparation of films or sheets containing cellulose nitrate and relates more particularly to the use of cellulose nitrate of comparatively low nitrogen content and of low viscosity characteristics in the preparation of films or sheets.

An object of our invention is to prepare films or sheets containing cellulose nitrate of low viscosity characteristics, and preferably of relatively low nitrogen content whereby films or sheets may be produced which have properties that are superior to those found in sheets or films heretofore made. Other objects of our invention will appear from the following detailed description.

Heretofore cellulose nitrate films have been prepared by spreading or flowing viscous solutions of the same onto metallic or other surfaces, and after suitable exposure to cause evaporation of the volatile solvents, the dry or partially dry film was stripped for use or other treatment.

However in this process, it has been necessary to employ a cellulose nitrate or pyroxylin of about 12% nitrogen content, produced by the reaction of a mixture of sulphuric acid and nitric acid on cellulose, without further treatment to alter the viscosity or solubility characteristics of the cellulose nitrate after such nitration. Films formed in this manner have been limited in their commercial application because of their lack of plasticity under heat and their sluggish response to cementing operations.

In order to overcome the difficulties when such cellulose nitrate was employed, it has been necessary to use large proportions of camphor or equivalent plastifiers and also certain modifiers such as fusel oil or similar high boilers,—all of which tended to distort the films or to impart to them an undesirable degree of softness.

We have discovered that all of these difficulties encountered in making a plastic film containing cellulose nitrate may be obviated by the use of a cellulose nitrate or pyroxylin of lower nitrogen content and of lower viscosity.

In accordance with our invention, we prepare films or sheets from solutions of cellu-

lose nitrate or pyroxylin of a comparatively low degree of nitration and having low viscosity characteristics, preferably lowering this viscosity by chemical and/or physical means after the process of nitration is completed. The solutions of such cellulose nitrate may be made in a suitable volatile solvent to which is added a plastifier and, if desired, a stabilizer such as urea. This solution, preferably after filtration, is cast or flowed onto a flat surface or on a wheel such as is used for forming films, and the volatile solvent is caused to evaporate preferably by means of a heated atmosphere. The amount of solution flowed onto the surface is such that it produces films or sheets ranging in thickness from that of ordinary films to that of the comparatively thick sheets which heretofore have been made by cutting from blocks of plastic masses of cellulose nitrate. The films are then stripped from the surface and are given any subsequent treatment desired.

The cellulose nitrate or pyroxylin to be employed in our process is preferably one that has a nitrogen content of 10.7 to 11.35% and preferably 11%. The viscosity characteristics of the cellulose nitrate employed is preferably from 10 to 75 seconds. This viscosity is determined by measuring the time required for a steel ball having a diameter of 3/32 of an inch to fall the distance of 11.44 inches through a solution maintained at a temperature of 25° C., which solution is formed by dissolving one part of the cellulose nitrate in 9 parts of a mixture of equal weights of 188° proof ethyl alcohol and acetone. This low viscosity cellulose nitrate may be made in any suitable manner known to the pyroxylin art. However we prefer to prepare it by treating a cellulose nitrate after it has been formed by nitration of cellulose with hot water under pressure in the presence of or the absence of chemical agents such as catalysts that promote the reduction of the viscosity characteristics of the cellulose nitrate.

Any suitable volatile solvent may be employed in making the solution, examples of which are acetone, a mixture of ethyl alcohol

or methyl alcohol with ether, or a mixture of ethyl alcohol or methyl alcohol with acetone.

- 5 While we prefer to employ camphor as the plastifier, other suitable plastifiers such as diethyl phthalate or dibutyl phthalate may be employed. The amount of plastifier used is generally within the range of that employed for making sheets from plastic compositions.
- 10 As an example of the quantity of plastifier that is suitable, it is pointed out that for 100 parts of cellulose nitrate 40 to 50 parts of camphor may be used.

15 By the use of our process, films or sheets may be produced which are clean and readily moldable and yet have all the desirable properties of films made from cellulose nitrate or pyroxylin having a nitrogen content of 12% and of normal viscosity. An important 20 application of our invention is the formation of comparatively thick films or sheets of pyroxylin. Heretofore the preparation of sheets or thick films by flowing solutions of the same on polished surfaces has been extremely difficult, if not impossible. Because 25 of the low viscosity characteristics of the cellulose nitrate employed, the solution of the same may be cast in such thickness, that the films or sheets resulting from the evaporation of the volatile solvent thereof have thicknesses equal to that of the thinner sheets formed by cutting from solid blocks of plastic composition. Thus by our process, flowed sheets may be formed that have a thickness 30 of .015 inch gauge—a result that has not been attainable heretofore.

35 The sheets or films produced by our process have smooth and highly polished surfaces and may be as readily shaped by molding and embossing as sheets formed by planing blocks of plastic masses containing cellulose nitrate. Unlike sheets formed by planing, the sheets made by our process are free of ploughed lines, so that even when heat or a solvent is applied to our films or sheets, the highly 40 glossed surfaces are unaffected. These sheets or films have a clarity and transparency superior to those heretofore made, have a high degree of plasticity, and may be readily cemented to other surfaces. Because of these 45 properties, they are eminently suited for all purposes for which films have been heretofore used, such as photographic films, and may also be put to the use to which planed sheets have been put. An important application 50 of the films or sheets produced by our process is in the making of laminated glass.

55 We are aware of the fact that varnish films have been formed on metallic or other surfaces by the application of solutions containing cellulose nitrate of reduced viscosity, say the so-called "½ second" viscosity cellulose nitrate. However the application of such solutions has had for its object the production of protective films that firmly adhere

to the surfaces, which films were not intended to be removed from such surfaces. Moreover even if such films were to be detached from the surfaces to which they are applied, they would be found to be very brittle and useless for any purpose. On the other hand, because of the nature of the cellulose nitrate, the solution and mode of procedure employed in our process, the film or sheet formed by our process is readily stripped from the supporting surface, it is intended to be used after separation from the supporting surface, and has the highly desirable properties above described.

60 As an example of one mode of carrying out our invention, a solution is made up as follows:—

|                                                                    | Parts  |
|--------------------------------------------------------------------|--------|
| Cellulose nitrate of 11% nitrogen content and 15 seconds viscosity | 100 85 |
| Camphor                                                            | 50     |
| Urea                                                               | 1      |
| Acetone                                                            | 400    |

65 This solution is carefully filtered to clarify the same and to remove foreign matter. The solution is flowed on the rim of a slowly rotating large wheel in required thicknesses and the acetone is caused to evaporate by exposure to the air. The films or sheets thus produced are stripped from the wheel.

70 It is to be understood that the foregoing detailed description is given merely by way of illustration and that many variations may be made therein without departing from the spirit of our invention.

75 Having described our invention what we claim and desire to secure by Letters Patent is:

1. Method of preparing films or sheets comprising applying a solution containing a volatile solvent and cellulose nitrate having a viscosity of 10 to 75 seconds and a nitrogen content of 10.7 to 11.35% to a surface, permitting the volatile solvent to evaporate and then stripping the film or sheet thus formed from the surface.

2. A flowed sheet or film containing cellulose nitrate of a viscosity of 10 to 75 seconds and having a nitrogen content of 10.7 to 11.35%.

3. A composition of matter adapted to be applied to a surface in the manufacture of films or sheets, containing cellulose nitrate having a viscosity of 10 to 75 seconds and a nitrogen content of 10.7 to 11.35% and a volatile solvent.

80 In testimony whereof, we have hereunto subscribed our names.

JAMES F. WALSH.

THOMAS E. ALCORN.

125

130